

June 14, 1960

W. HELLING ET AL

2,940,228

APPARATUS FOR POLISHING METALS

Original Filed July 3, 1956



FIG.1



FIG.2



FIG.3

INVENTOR:  
Werner Helling  
and  
BY: Heinrich Neunzig  
Michael S. Striker  
ATTORNEY

## 1

2,940,228

## APPARATUS FOR POLISHING METALS

Werner Helling, Grevenbroich, and Heinrich Neunzig, Gindorf, near Grevenbroich, Germany, assignors to Vereinigte Aluminum-Werke Aktiengesellschaft, Bonn, Germany

Original application July 3, 1956, Ser. No. 595,792. Divided and this application Aug. 22, 1957, Ser. No. 679,685

Claims priority, application Germany July 8, 1955

7 Claims. (Cl. 51—263)

The present invention relates to an apparatus for polishing metals and, more specifically, it relates to an apparatus for forming a highly glossy surface on metal bodies.

The present application is a division of our copending application Serial No. 595,792, filed on July 3, 1956 and entitled "Method and Apparatus for Polishing Metals."

Customarily wet-polishing operations are carried out with polishing apparatus having polishing wheels, the working surfaces of which are covered with cloth or felt, or with polishing wheels which in their entirety consist of cloth or felt (so-called flexible buffering wheels). Furthermore, textile bands are also used for this purpose. By employing any of the aforementioned polishing members it is not possible to achieve an especially high gloss, to the contrary there always remains microscopically fine scratches, which for instance give to such polished metal surface an undesirable cloudy luster. It is a further disadvantage of the above-discussed devices that the textile materials absorb and retain only small quantities of the polishing fluid. Consequently, textile covered polishing wheels cause spinning off of considerable quantities of the polishing fluid due to the centrifugal forces created by the rotating polishing wheel. The spun-off polishing fluid circulates without useful effect.

It is therefore an object of the present invention to overcome the aforementioned disadvantages of conventional wet-polishing apparatus.

It is another object of the present invention to provide a wet-polishing apparatus including a polishing member capable of absorbing and retaining relatively large quantities of polishing fluid.

It is a further object of the present invention to provide a wet-polishing apparatus including a rotating polishing member which may be rotated at a very low surface speed while still effectively polishing metal surfaces.

It is still another object of the present invention to provide a wet-polishing apparatus, during operation of which the losses on polishing fluid are reduced to a minimum.

It is yet another object of the present invention to provide in a wet-polishing apparatus a polishing member capable of imparting a very high gloss to metal surfaces.

Other objects and advantages of the present invention will become apparent from a further reading of the description and of the appended claims.

With the above and other objects in view, the present invention mainly comprises in a polishing apparatus adapted to wet-polish the surface of a metal body, a polishing member having a working outer portion consisting of a porous plastic material.

It should be noted that throughout the present application and claims the term "porous" is meant to indicate open pores or a mixture of open and closed pores, but does not include exclusively closed pores. The term "porous" is further meant to indicate that the structure of the porous material is such that a liquid can pass through interconnected open pores throughout the entire body of the material.

According to a preferred embodiment of the present

## 2

invention, the same includes a polishing apparatus for wet-polishing the surface of a metal body, comprising, in combination, a rotatable polishing disc consisting essentially of a porous plastic material belonging to the group consisting of natural and synthetic rubbers, viscose, urea resins, phenolic resins, polyurethanes, polystyrenes and polyvinyl chlorides, the size of the pores in the porous plastic material being between about 100 and 1,000 microns, rotating means for rotating the polishing disc and including a rotatable shaft having a hollow perforated portion, the porous disc being mounted on the hollow perforated shaft portion, collecting means for collecting polishing fluid separating from the polishing disc during operation of the polishing apparatus, and pumping means 15 communicating with the collecting means and with the hollow perforated shaft portion for passing polishing fluid from the collecting means into the hollow perforated shaft portion, whereby upon rotating of the shaft polishing fluid will pass through the perforations of the hollow shaft portion into the porous polishing wheel and to the outer working surface thereof due to the centrifugal force exerted by the rotating porous polishing wheel.

Surprisingly, it has been found according to the present invention that a considerable increase in the quality of 25 the polish and gloss of aluminum and aluminum alloy surfaces as well as of other metal and metal alloy surfaces can be obtained by employing instead of textile polishing wheels, polishing wheels or bands which have at least a working surface made of porous plastic materials. 30 Elastomers such as natural or synthetic rubber, viscose, urea or phenolic resins, polyurethanes, polystyrenes, polyvinyl chlorides and others may be employed. The polishing wheels or bands or other polishing members may be formed completely of such porous plastic materials or may be entirely or in part covered with the same. 35 Preferably, materials having open pores of a size between 100 and 1,000 microns are used.

A further advantage of employing such porous elastomers consists in the reduction of the required speed of the 40 wheels or bands as compared with the speed required when using the customary felt or cloth polishing members. Consequently, the centrifugal forces are less, the polishing liquid is absorbed into the pores of the polishing member and retained therein without being spun off in large quantities due to excessive centrifugal forces.

The discs or wheels made of such synthetic or natural 45 elastomers, or at least having working surfaces covered with the same, absorb the polishing fluid and retain a large portion of the same, since the centrifugal forces, due to the slow surface speed do not cause any spinning-off of polishing fluid. It is a further advantage of the 50 polishing members according to the present invention that the metal or metal alloy body which is to be polished can be strongly pressed onto the working surface of the disk which can be formed of commensurate width. 55 Thereby the metal body will partially be embedded into the surface of the plastic porous disk under temporary deformation of the disk. In this manner it is possible also to polish metal bodies which have an uneven surface such as reliefs or portions of mountings, instruments and 60 the like, since the polishing disc acts on a larger portion of the surface of the metal body. Thereby too, the polishing fluid is for all practical purposes retained in the porous plastic wheel and is not spun-off.

The surface speed or rim speed of polishing wheels or 65 bands made of porous elastomers can be as low as between 2 and 3 meters per second. At such low speed many of the dangers which otherwise exist when polishing uneven bodies are avoided. Customary polishing discs having textile covered working surfaces or polishing bands of customary textile material have to be operated 70 at considerably higher speeds such as speeds of between

20 and 30 meters per second since otherwise the polishing effect can not be obtained. The danger, as is well known, consists in the possibility that the metal body may attach itself to the fast moving polishing member and may then be thrown off the same. Consequently, the low speed porous plastic polishing wheels or bands according to the present invention are especially suitable for polishing metal bodies of complicated uneven configuration. Accordingly, the previously existing difficulties in the wet-polishing of metal bodies with suspensions of solid particles in a liquid medium can be avoided by employing the polishing members of the present invention which have at least working surfaces made of porous natural or synthetic elastomers.

The novel features which are considered as characteristic for the invention are set forth in particular in the appended claims. The invention itself, however, both as to its construction and its method of operation, together with additional objects and advantages thereof, will be best understood from the following description of specific embodiments when read in connection with the accompanying drawings, in which:

Fig. 1 is a schematic elevational view of an embodiment of the apparatus of the present invention;

Fig. 2 is a schematic elevational view of another embodiment of an apparatus according to the present invention; and

Fig. 3 is still another schematic elevational view of a different embodiment of the present invention.

Referring now to the drawing and particularly to Fig. 1, a motor 1 is shown driving a shaft 2. On shaft 2 is mounted a polishing wheel or disc 3 having an outer working portion 4, the working surface of which will come in contact with the metal body to be polished. Working portions 4 of polishing member 3 is made of a porous plastic material adapted to apply a polishing fluid to the metal body. Polishing fluid squeezed out of the porous plastic working portion of polishing member 3 is collected in a vessel 5 and pumped by pump 6 through conduit 7, from the open end of which the polishing fluid is again introduced to the porous plastic working portion 4 of polishing member 3. The polishing fluid, while passing through conduit 7 is cooled by cooling means 8. Motor 1 and shaft 2 constitute the rotating means, conduit 7 is an embodiment of the liquid-introducing means, collecting means are represented by vessel 5, and pump 6 together with the conduit connecting vessel 5 with pump 6 represent the pumping means.

The different embodiment shown in Fig. 2 includes a hollow shaft portion 11 as part of the rotating means, on which is mounted a polishing wheel 12 which is made entirely of a porous plastic material. Brackets 13 are provided for giving additional support to polishing member or wheel 12. Polishing fluid is pumped through conduit 14 into hollow shaft 11 and enters the porous plastic polishing wheel 12 through hollow perforated shaft portion 11. Polishing fluid squeezed off the working surface of polishing wheel 12 when the same is in contact with a metal body to be polished, is collected in vessel 5 from where it flows to pump 6 for being recirculated through conduit 14. Cooling means 8 are provided for controlling the temperature of the polishing fluid.

The embodiment shown in Fig. 3 differs from the embodiment shown in Fig. 1 by having a polishing band or belt 21 provided with a working portion 22 formed of a porous plastic material.

The operation of the apparatus of the present invention may for instance be as follows:

A disc made of finely porous polyurethane, having a width of about 100 mm. and a diameter of about 300 mm. is mounted on a grinding head in a manner similar to the mounting of a grinding wheel. The pores of the polyurethane wheel preferably have a size of between 100 and 1,000 microns. The polyurethane polishing

wheel is mounted on a shaft by means of two lateral brackets preferably made of wood, hard rubber or a suitable strong synthetic material and having rounded edges. The polishing wheel is rotated with about 160 turns per minute corresponding to a peripheral velocity of about 2.5 meters per second. The wheel is completely saturated with polishing fluid consisting for instance of a suspension of aluminum oxide hydrate or alumina in water to which a small quantity of a commercial wetting agent has been added. The metal bodies to be polished are firmly pressed against the polishing wheel so that they penetrate to some extent into the resilient working surface thereof. Thereby polishing fluid is pressed out of the polishing wheel and due to the low velocity this

15 fluid remains for a short period of time on the surface of the metal body from which the fluid slowly drops into a collecting vessel. It should be noted that due to the low velocity and correspondingly small centrifugal force, the polishing fluid is not spun off the polishing wheel. Consequently, it is not necessary to provide baffle sheets or other protective devices to catch polishing fluid spraying off the apparatus. The polishing fluid dropping from the metal body is collected and returned to the polishing wheel as indicated in the description of the drawing.

20 The porous plastic materials of which the entire polishing wheel may be formed are also well suited for conducting the polishing fluid to the working surface of the polishing wheel, for instance by providing a hollow shaft on which the polishing wheel is mounted and through which the polishing fluid is supplied. This has been illustrated in Fig. 2. The polishing fluid may also be pressed into the small intervening space between several polishing wheels which are mounted next to each other. In this manner, too, the polishing fluid can be supplied to the working 25 surface of the polishing wheel.

25 The difference in gloss obtained on metal surfaces of the same composition and under otherwise equal conditions by replacing the conventional textile polishing member of a wet-polishing apparatus with the porous plastic polishing member according to the present invention is illustrated in Table I further below.

30 The examples which are summarized in Table I are given as illustrative only, the present invention, however, not being limited to any of the specific details of the examples.

#### EXAMPLE 1

An aluminum magnesium alloy body including 0.01% Cu, 0.011% Zn, 0.066% Si, 0.033% Fe, 0.002% Mn, 1.92% Mg and the balance aluminum, in the form of a 35 normal commercial sheet with a cold rolled finished surface, was first dry-polished with a polishing paste consisting of 66 parts of finely sub-divided alumina, 26 parts of stearin, 6 parts of montan wax, and 2 parts of petroleum jelly. The dry polishing was carried out with a 40 flexible polishing wheel made of nettle cloth, having a diameter of 300 mm. and a width of 40 mm. The dry polishing was carried out at a circumferential speed of 50 meters per second for a period of 2 minutes. The dry polished metal body was then pickled by immersion 45 for 30 seconds in a 10% aqueous sodium hydroxide solution having a temperature of 55° C., subsequent rinsing with water followed by neutralization by immersion for a short period of time in 20% aqueous nitric acid at room temperature.

50 The thus pre-treated metal body was then wet polished with a conventional textile polishing wheel. A polishing fluid prepared by diluting 300 cubic centimeters of a commercial suspension of polishing alumina (Number 3 of the firm Jean Wirtz, Dusseldorf) with 1 liter of water and adding thereto 1.3 grams of an oxyethylmethyl cellulose of medium viscosity (Tylose SL 400 made by Kalle & Co., Wiesbaden-Bierbrich), was used.

55 The flexible polishing wheel consisted of several layers of absorbent soft cotton which had been sewn together. The diameter of the polishing wheel was 300 mm. and the

width 40 mm. The circumferential speed of the rotating polishing wheel was 20 meters per second. The above-described polishing fluid was sprayed onto the polishing wheel. Wet polishing was carried out for a period of 10 minutes. Thereafter, the metal body was sprayed with water.

Finally, the metal body was anodically oxidized for 10 minutes in 20% aqueous sulfuric acid at 18° C. with a current density of 1.5 amperes per 100 square centimeters. The thus obtained oxide layer had a thickness of approximately 5 microns.

A parallel experiment was carried out exactly as described above, with the only exception that the wet-polishing was accomplished with a porous plastic polishing wheel in the following manner:

The same wet-polishing liquid was used as described above. The polishing wheel was made of finely porous polyurethane (Moltopren 0.055 blue, thickness 10 centimeters made by Pongs & Co., Aachen). The wheel had a diameter of 300 mm. and a width of 100 mm. and was mounted on a grinding head in a similar manner as a grinding wheel. The wheel was rotated with 160 revolutions per minute, corresponding to a circumferential speed of about 2.5 meters per second. The wheel was completely saturated with polishing fluid, the polishing fluid which dropped off the wheel and/or the metal body was caught and recirculated to the polishing wheel. Polishing was carried out for 4 minutes.

#### EXAMPLE 2

Parallel experiments were carried out as described in Example 1, however, the sheets which were thus-treated were made of an aluminum magnesium alloy containing 99% of high purity aluminum (99.99% aluminum) and 1% magnesium.

#### EXAMPLE 3

Commercial cold rolled brass sheets were first dry-polished and thereafter wet-polished either with a conventional cloth polishing wheel or with a porous plastic polishing wheel, as described above.

In all of the above-described experiments, the total and specular reflection of the finished product was measured and the following values were found:

Table I

|                                     | Reflection<br>Specular,<br>Percent | Total,<br>Percent |
|-------------------------------------|------------------------------------|-------------------|
| Example I—Textile Polishing Wheel   | 70.3                               | 82.4              |
| Porous Plastic Wheel                | 79.6                               | 89.9              |
| Example II—Textile Polishing Wheel  | 77.3                               | 80.1              |
| Porous Plastic Wheel                | 81.4                               | 86.9              |
| Example III—Textile Polishing Wheel | 69                                 | 78                |
| Porous Plastic Wheel                | 72                                 | 85                |

It is apparent from the results shown in Table I that considerably higher reflection values are obtained with the polishing apparatus according to the present invention as can be obtained under otherwise equal conditions with conventional polishing apparatus.

It will be understood that each of the elements described above, or two or more together, may also find a useful application in other types of polishing apparatus differing from the types described above.

While the invention has been illustrated and described as embodied in a polishing apparatus, it is not intended to be limited to the details shown, since various modifications and structural changes may be made without departing in any way from the spirit of the present invention.

Without further analysis, the foregoing will so fully reveal the gist of the present invention that others can by applying current knowledge readily adapt it for various applications without omitting features that, from the standpoint of prior art, fairly constitute essential charac-

teristics of the generic or specific aspects of this invention and, therefore, such adaptations should and are intended to be comprehended within the meaning and range of equivalence of the following claims.

5. What is claimed as new and desired to be secured by Letters Patent is:

1. In a polishing apparatus for wet polishing metal bodies so as to obtain a glossy surface thereon, in combination, a polishing member having a continuous outer working portion consisting essentially of an open-cell, porous, elastomeric plastic material; feeding means for feeding a polishing suspension onto said outer working portion of said polishing member at a portion thereof spaced from the area of simultaneous contact between a

15 metal body to be polished and said polishing member, to be absorbed by the same and to be squeezed out of the same at a polishing surface thereof when the article to be polished is pressed against said polishing surface; collecting means for collecting polishing fluid squeezed out of said polishing member and for returning collected polishing fluid to said feeding means; and automatic means for rotating said outer working portion of said polishing member at a circumferential speed sufficiently low to substantially prevent the spinning off of polishing 25 suspension due to centrifugal force, relative to and in contact with the surface of a metal body to be polished.

2. In a polishing apparatus for wet polishing metal bodies so as to obtain a glossy surface thereon, in combination, a rotating polishing member having a continuous

30 outer working portion consisting essentially of an open-cell, porous, elastomeric plastic material; feeding means for feeding a polishing suspension onto said outer working portion of said polishing member at a portion thereof spaced from the area of simultaneous contact between a

35 metal body to be polished and said polishing member, to be absorbed by the same and to be squeezed out of the same at a polishing surface thereof when the article to be polished is pressed against said polishing surface; collecting means for collecting polishing fluid squeezed out of said polishing member and for returning collected polishing fluid to said feeding means; cooling means between communicating with said collecting means and said feeding means for cooling polishing suspension flowing from said collecting means to said feeding means and 40 automatic means for rotating said outer working portion of said polishing member at a circumferential speed sufficiently low to substantially prevent the spinning off of polishing suspension due to centrifugal force, relative to and in contact with the surface of a metal body to be polished.

3. In a polishing apparatus for wet polishing metal bodies so as to obtain a glossy surface thereon, in combination, a polishing member having a continuous outer working portion consisting essentially of an open-cell,

55 porous, elastomeric plastic material; feeding means for feeding a polishing suspension onto said outer working portion of said polishing member at a portion thereof spaced from the area of simultaneous contact between a

60 body to be polished and said polishing member, to be absorbed by the same and to be squeezed out of the same at a polishing surface thereof when the article to be polished is pressed against said polishing surface; and automatic means for moving said outer working portion of said polishing member and the surface of a metal body 65 to be polished.

4. In a polishing apparatus for wet polishing metal bodies so as to obtain a glossy surface thereon, in combination, a polishing member having a continuous outer working portion consisting essentially of an open-cell, porous, elastomeric plastic material selected from the group consisting of natural and synthetic rubbers, viscose, urea resins, phenolic resins, polyurethanes, polystyrenes and polyvinyl chlorides and formed with interconnected open pores having diameters of between about 70 100 and 1000 microns; feeding means for feeding a pol-

ishing-suspension onto said outer working portion of said polishing member at a portion thereof spaced from the area of simultaneous contact between a metal body to be polished and said polishing member, to be absorbed by the same and to be squeezed out of the same at a polishing surface thereof when the article to be polished is pressed against said polishing surface; collecting means for collecting polishing fluid squeezed out of said polishing member and for returning collected polishing fluid to said feeding means; and automatic means for movement between rotating said outer working portion of said polishing member at a circumferential speed sufficiently low to substantially prevent the spinning off of polishing suspension due to centrifugal force, relative to and in contact with the surface of a metal body to be polished.

5. In a polishing apparatus for wet polishing metal bodies so as to obtain a glossy surface thereon, in combination, a polishing disc consisting essentially of an open-cell, porous, elastomeric plastic material and having a continuous outer working portion; feeding means for feeding a polishing suspension onto said outer working portion of said polishing disk at a portion thereof spaced from the area of simultaneous contact between a metal body to be polished and said polishing member, to be absorbed by the same and to be squeezed out of the same at a polishing surface thereof when the article to be polished is pressed against said polishing surface; collecting means for collecting polishing fluid squeezed out of said polishing member and for returning collected polishing fluid to said feeding means; and automatic means for rotating said polishing disc at a circumferential speed of up to about 3 meters per second relative to and in contact with the surface of a metal body to be polished.

6. In a polishing apparatus for wet polishing metal bodies so as to obtain a glossy surface thereon, in combination, a polishing belt consisting essentially of an open-cell, porous, elastomeric plastic material and having a continuous outer working portion; feeding means for feeding a polishing suspension onto said outer working portion of said polishing belt at a portion thereof spaced from the area of simultaneous contact between a metal body to be polished and said polishing member, to be

5 absorbed by the same and to be squeezed out of the same at a polishing surface thereof when the article to be polished is pressed against said polishing surface; collecting means for collecting polishing fluid squeezed out of said polishing member and for returning collected polishing fluid to said feeding means; and automatic means for moving said polishing belt at a speed of up to about 3 meters per second relative to and in contact with the surface of a metal body to be polished.

10. 7. In a polishing apparatus for wet polishing metal bodies so as to obtain a glossy surface thereon, in combination, a rotating polishing member consisting essentially of an open-cell, porous, elastomeric plastic material selected from the group consisting of natural and synthetic rubbers, viscose, urea resins, phenolic resins, polyurethanes, polystyrenes and polyvinyl chlorides and formed with interconnected opened pores having diameters of between about 100 and 1000 microns; means for feeding a polishing suspension to said polishing member at a portion thereof spaced from the area of simultaneous contact between a metal body to be polished and said polishing member, to be absorbed by the same and to be squeezed out of the same at a polishing surface thereof when the article to be polished is pressed against said polishing surface; and means for rotating said polishing member at a circumferential speed of between 2 and 3 meters per second relative to and in contact with the surface of a metal body to be polished.

30 References Cited in the file of this patent

UNITED STATES PATENTS

|           |                 |               |
|-----------|-----------------|---------------|
| 490,808   | Kelley          | Jan. 31, 1893 |
| 1,975,451 | Dunaway         | Oct. 2, 1934  |
| 2,221,173 | Gutsell         | Nov. 12, 1940 |
| 2,268,403 | Kingman         | Dec. 30, 1941 |
| 2,328,998 | Radford         | Sept. 7, 1943 |
| 2,352,146 | Desenberg       | June 20, 1944 |
| 2,609,347 | Wilson          | Sept. 2, 1952 |
| 2,646,655 | Laverdissé      | July 28, 1953 |
| 2,764,856 | Steen et al.    | Oct. 2, 1956  |
| 2,804,728 | Politzer et al. | Sept. 3, 1957 |